

Nov. 22, 1932.

E. ROIRANT

1,888,393

PROCESS FOR PUSHING GLASS BOTTLES

Filed March 12, 1931 2 Sheets-Sheet 1

Fig.1.



Fig.2.



Fig.3.



E. Roirant  
INVENTOR

By: Marks & Elz, A.T.T.S.

Nov. 22, 1932.

E. ROIRANT

1,888,393

PROCESS FOR PUSHING GLASS BOTTLES

Filed March 12, 1931 2 Sheets-Sheet 2

Fig.4.



Fig.5.



Fig.6.



Fig.7.



E. Roirant  
INVENTOR

By: *Mauris Allen* *AT&T*

## UNITED STATES PATENT OFFICE

EMILE BOIRANT, OF PARIS, FRANCE, ASSIGNOR TO SOCIÉTÉ ANONYME D'ÉTUDES ET DE CONSTRUCTIONS D'APPAREILS MÉCANIQUES POUR LA VERRERIE, OF PARIS, FRANCE

## PROCESS FOR PUSHING GLASS BOTTLES

Application filed March 12, 1931, Serial No. 522,097, and in France April 17, 1930.

The operation known as "pushing" bottles is carried out in an auxiliary apparatus in which the blown bottle is placed on leaving the finishing mould. Vain attempts have been made to avoid this supplementary handling and operation by trying to effect the "pushing" in the finishing mould, immediately after blowing and by the same means as that employed in the auxiliary apparatus.

10 It is known that these means consist in substituting for the bottom of the finishing mould, after the bottle is blown, a device called a "pusher" intended to press in the glass at the bottom and to give it the required form.

The result obtained has always been indifferent; the defects noted in a constant manner, consist in a bad disposition of the thickness of the glass constituting the "push" and 20 in rents or cracks of the exterior surface of this "push".

It will suffice to explain the causes of these defects to cause the process employed to eliminate them to be understood, a process 25 which constitutes the subject of the present invention.

Figures 1 and 2 represent the means known up to the present to produce the "push" in the finishing mould.

30 Figure 3 shows the push thus produced and the defects that may be noted in it.

Figures 4, 5 and 6 show the new phases of "pushing", the succession of which constitutes the subject of the present invention.

35 Figure 7 shows a modification of the same proposed means.

Figure 1 shows in section the lower part of the bottle F such as it is blown upon the bottom 1 of the finishing mould, which may have 40 any desired profile.

It is a fact that experience has always allowed to be noticed, that the thickness of the glass forming the bottom is never regular. The central part *o* is always much more thick 45 than the periphery *p*. This anomaly is due to the blowing, which first applies centrally the glass upon the central part of the finishing bottom 1, aided in so doing by the weight, then subsequently a drawing out is produced towards the periphery, whence a continuous

diminution of thickness and so much the more if the bottom has a large diameter.

Figure 1 shows, with guarded proportions, the variation of thickness noticed on many occasions.

55 The blowing has equally another consequence: when the glass is applied to the metallic surface of the bottom 1, the surface of the glass in contact with the metal is suddenly cooled and becomes very rigid whilst the interior surface retains to a considerable extent its original temperature.

60 In order to effect the "pushing" there is rapidly substituted for the finishing bottom 1 a pusher 2 (see Fig. 2) having a movement 65 in the direction of the arrow *f*.

65 The result, shown in Fig. 3, is such that the part A B C is made thin at the end whilst the periphery AD, C E, having a thickness 70 approximately equal to the original thickness, is cracked or crackled, as indicated at *g*.

75 These particularities are easily explainable: during the time that the pusher 2 has been substituted for the bottom 1, the central part which is very thick and in consequence very hot has been able to reheat, in a certain measure, the corresponding exterior skin, previously cooled by the metallic contact.

80 When the pusher is put into action to push in the glass, it has found the central portion much more malleable than the periphery and all this central portion is stretched easily whilst the neighbouring parts have resisted the traction to which they were submitted.

85 The exterior skin of the peripheral region, insufficiently reheated, is then crackled under the effort, whence the result shown in Fig. 3.

90 It appears therefore that these difficulties are the consequence of the diversity of the thickness of the bottom of the bottle (Fig. 1), causing a thermic diversity which does not permit the bottom of the bottle to be deformed regularly to transform it into a pushed bottom.

95 These are difficulties which have necessitated the known employment of an auxiliary apparatus, not for modifying the method of pushing—which is exactly the same—but to allow, in fact, by sufficient lapse of time between the blowing and the "pushing", a uni-

formity of temperature of the glass at the bottom or rather a tendency to this uniformity for the purpose of enabling the pushing to be effected in the best conditions.

It is certain that the same result might be obtained in the finishing mould if sufficient time were allowed, but the time required is relatively considerable and the diminution of production which would follow would render prohibitive this method of working.

10 The present invention consists in employing means which realize, in the time available between the moment of blowing and the moment of expulsion of the bottle from the mould, the conditions required for obtaining a "push" free from the usual defects.

15 These means consist in acting at the same time upon the distribution of the glass at the bottom and regulating the temperature of this glass.

20 In the first phase illustrated in Fig. 4, the bottom of the finishing mould,—after it has served for blowing the bottle the bottom of which has the same defect of distribution as in Fig. 1 (thicker glass at the centre *o* than upon the periphery *p*),—is moved into an intermediate position 3. It is also possible, at least theoretically, to leave the bottom 3 in the position which it occupies during blowing and to move the bottle, the object being, 25 in both cases, to separate the bottom of the bottle from the bottom of the finishing mould.

Fig. 5 shows a second phase in which the bottom of the bottle, either under the action 30 of its weight, or under the action of a light puff of air, has taken the bent position indicated in this figure.

It is easily understood that for the same reasons as those which have been previously 35 set forth, and which proved that the central hotter part was stretched towards the top under the action of the "pusher", this same part is stretched downwards at *o'*, thus re-establishing the equality of thickness; this 40 re-establishment depends upon the amount of separation of the bottom of the bottle from the bottom of the finishing mould.

It will be equally understood that this 45 second phase results in a thermic action which is transferred by a new cooling of the central hotter part coming to rest upon the metallic bottom which has a cooling action, whilst the cooler outer skin of the peripheral part, tends to become heated by auto-reheating because it is no longer in contact with metal.

These particularities will therefore permit, 50 when the pusher 2 is substituted for the finishing bottom the presentation to this pusher 55 of a bottom realizing the indispensable conditions for the operation of "pushing" and at the same time will avoid the irregular stretching and the cracks noted in the first method (see Fig. 6).

60 Fig. 7 shows a modification of the new

process. It consists in substituting the "pusher" for the finishing bottom immediately after blowing, in arresting the "pusher" at a certain distance from the bottom of the bottle, in a manner to allow the phase of regulating the thickness and of regulating the heat of the bottom of the bottle to be accomplished before "pushing", then finally executing the operation of pushing.

70 Experience has proved that the time occupied in this preliminary phase of pushing does not slow down the usual production and that it corresponds approximately to the indispensable time necessary for cooling, after blowing, the bottle in the interior of its mould 80 before it is expelled therefrom.

I claim.

1. A process of "pushing" bottles in the interior of a finishing mould, which consists, 85 after blowing of the bottle, in separating the bottom of the finishing mould and the bottom of the bottle from each other, then in allowing the central portion of the bottom of the bottle to sag and rest during a suitable period of time on the corresponding part of the finishing bottom, in substituting the "pusher" for the finishing bottom, and finally in effecting the "pushing" of the bottom of the bottle.

90 2. A process of "pushing" bottles in the interior of a finishing mould, which consists, after blowing of the bottle, in removing to a suitable distance the bottom of the finishing mould, leaving the bottle stationary, then in allowing the central portion of the bottom 100 of the bottle to sag and rest during a suitable period of time on the corresponding part of the finishing bottom, in substituting the "pusher" for the finishing bottom, and finally in effecting the pushing of the bottom of the bottle.

95 3. A process of "pushing" bottles in the interior of a finishing mould, which consists, after blowing of the bottle, in removing the bottle to a suitable distance, leaving the finishing bottom stationary, then in allowing the central portion of the bottom of the bottle to sag and rest during a suitable period of time on the corresponding part of the finishing bottom, in substituting the "pusher" for the finishing bottom, and finally in effecting the pushing of the bottom of the bottle.

100 4. A process of "pushing" bottles in the interior of a finishing mould, which consists, after blowing of the bottle, in separating the bottom of the finishing mould and the bottom of the bottle from each other, then in allowing the central portion of the bottom of the bottle to sag by gravity and rest during a suitable period of time on the corresponding 115 part of the finishing bottom, in substituting the "pusher" for the finishing bottom, and finally in effecting the "pushing" of the bottom of the bottle.

120 5. A process of "pushing" bottles in the interior of a finishing mould, which consists, after blowing of the bottle, in separating the bottom of the finishing mould and the bottom of the bottle from each other, then in allowing the central portion of the bottom of the bottle to sag by gravity and rest during a suitable period of time on the corresponding 125 part of the finishing bottom, in substituting the "pusher" for the finishing bottom, and finally in effecting the "pushing" of the bottom of the bottle.

130 5. A process of "pushing" bottles in the interior of a finishing mould, which consists, after blowing of the bottle, in separating the bottom of the finishing mould and the bottom of the bottle from each other, then in allowing the central portion of the bottom of the bottle to sag by gravity and rest during a suitable period of time on the corresponding part of the finishing bottom, in substituting the "pusher" for the finishing bottom, and finally in effecting the "pushing" of the bottom of the bottle.

- terior of a finishing mould, which consists, after the blowing of the bottle, in separating the bottom of the finishing mould and the bottom of the bottle from each other, then in effecting a slight blowing for causing the central part of the bottle to sag and rest on the corresponding part of the finishing bottom, in substituting the "pusher" for the finishing bottom, and finally in effecting the pushing of the bottom of the bottle.
- 10 6. A process of "pushing" bottles in the interior of finishing mould, which consists, after blowing of the bottle, in immediately substituting the "pusher" for the finishing bottom, in stopping the "pusher" at a certain distance from the bottom of the bottle, in allowing the central part of the bottom of the bottle to sag and rest on the "pusher" and finally in effecting after a suitable time the "pushing" of the bottom of the bottle.
- 15 7. A process for the manufacture of bottles with "pushed" bottom in a finishing mold, comprising finishing molds adapted to be displaced axially, characterized by the fact that after blowing the bottle in the finishing mold with a flat bottom, the bottom of the mold is removed to such an extent that the bottle bottom sags by reason of the softening resulting from its internal heat is only in contact through its central part with the bottom of the mold brought behind so that by replacing the flat finishing mold by a pusher and by advancing this pusher, the "pushing" is effected.
- 20 8. A process according to claim 7, characterized by the fact that immediately after the blowing of the bottle in the finishing mold with a flat bottle bottom, the flat bottom of the finishing mold is replaced by a pusher at the point on which the central part of the sagging bottom of the bottle rests whereupon by advancing the pusher, the "pushing" is effected.

The foregoing specification of my "Improved process for "pushing" glass bottles";  
45 signed by me this 27th day of February 1931.  
EMILE ROIRANT.